

## UNITED STATES PATENT OFFICE

2,364,792

## PRODUCTION OF ZEIN COATING

Albert L. James, Tenafly, N. J., assignor to Corn Products Refining Company, New York, N. Y., a corporation of New Jersey

No Drawing. Application January 31, 1942,  
Serial No. 429,136

6 Claims. (Cl. 106—153)

This invention relates to the production of zein coatings and the like, and the primary objects of the invention are to increase the water resistance of such coatings and also to shorten the "curing time," that is, the time required for bringing the coating to a state in which it is relatively hard and water resistant.

A specific object of the invention is to provide an aqueous zein dispersion which may be used, as an adhesive, in the place of casein adhesives, in the clay coating of paper for lithographing purposes, whereby the coating operation is simplified and the cost of the same reduced, the water resistance of the coating improved and, more particularly, the curing time is very substantially shortened. The shortened curing time is important in clay coating for lithography as it is often desirable to lithograph paper within a short time after it has been coated; and, usually, the coated paper is wetted with water before being subjected to the lithographing procedure, and, therefore, must be water-resistant at that time.

The following specific examples give instances of the reduction to practice of the invention, in certain preferred embodiments. It will be understood, however, that the specific examples are purely typical and illustrative. The invention is not limited to the particular operating data given therein. It is the intention to cover all equivalents and also all modifications within the scope of the hereto appended claims. In the examples, ranges are given in parentheses. These ranges are practical, not critical, unless particularly so specified. In the examples the proportions are given in parts by weight, unless otherwise specified.

*Example 1.*—382 parts of zein (commercial zein containing the usual amount of water) is mixed with 1400 parts of water (1300 or over). To this is added first 75 parts (25 to 150 parts) of 85% sulfonated castor oil, containing, that is, 15% of water, and then 215 parts (150 to 350 parts) of a caustic soda solution consisting of 15 parts of sodium hydroxide dissolved in 200 parts of water. At this stage the zein is completely dissolved, or at least forms a dispersion which closely approximates a solution. To this solution or dispersion is added, slowly and with rapid agitation, a lead acetate solution made up of 20 parts of lead acetate (5 to 40 parts) and 200 parts of water.

The dispersion or solution made as above and consisting of approximately 2092 parts, is mixed with 2250 parts (1800 to 4500 parts) of clay, or its equivalent, and 2000 parts (1200 to 5000 parts)

of water. The paper is coated with this clay slurry and the sheets air-dried or dried at a suitable elevated temperature such as 150° F. This process will give a tenacious coating which will become in a high degree, and almost immediately, water resistant.

*Example 2.*—The following ingredients are mixed together according to the procedures indicated in Example 1, viz.: zein 17 parts, water 60 parts (20 parts to 60 parts), sulfonated talloil containing about 37% of water 3.4 parts (2 parts to 10 parts), caustic potash 0.8 part (0.51 part to 1.2 parts), lead acetate 0.85 part (0.35 part to 3.0 parts), clay 100 parts (50 parts to 200 parts).

15 In place of lead acetate it is possible to use any water soluble salt of a weak acid, such as acetic or formic acid. Examples are the acetates and formates of aluminum, barium, calcium, magnesium, tin, zinc and copper. Metal salts of strong acids should not be used, since they tend to precipitate the zein to such an extent that it is not readily redissolved by the excess of caustic soda. It is the lead acetate or its equivalent which appears to give the coating the capacity to develop a high degree of water resistance in a short period of time.

20 In the zein dispersion of the present invention, the primary dispersing agent is caustic soda. The sulfonated oil appears to be a secondary zein dispersing agent which brings about a more thorough dispersion in the water of the alkali dissolved zein. Furthermore, alkali solutions of zein are unstable tending to jell within a short time. The sulfonated oil acts to stabilize the alkali-zein solution or dispersion until such time as it may be used.

25 Any sulfonated oil which is capable of dispersing the zein and which is of such character that it will not be precipitated by the lead acetate in the presence of the excess of caustic soda, may be used in place of the sulfonated castor oil or talloil which latter, however, are preferred, especially the sulfonated talloil. In fact, any of the zein dispersing agents disclosed in application 45 of Albert Luther James, Serial No. 351,274, filed August 3, 1940, may be used in place of the sulfonated oils provided such zein dispersants have the property of not being precipitated by the presence of the lead acetate, or its equivalent. This excludes rosin size for the reason that rosin size, being a sodium soap of rosin, interacts with a metal salt, such as lead acetate, to form a metal rosin soap, for example, lead rosin soap, which is highly insoluble and would, therefore, bring about the precipitation of the rosin.

from the solution. For similar reasons soaps of the fatty acids cannot be used effectively as secondary zein dispersants in accordance with the present invention.

In place of caustic soda (sodium hydroxide) any alkali may be used which is capable of dispersing zein in water. Examples are potassium hydroxide, and compounds of ammonium hydroxide with caustic alkalies, and trisodium phosphate. Ammonium hydroxide alone is not effective, evidently because the pH of aqueous ammonia solutions is not high enough to bring about zein dispersion.

The term "clay," as used herein, is intended to cover any argillaceous or other earthy material commonly used for coating paper.

I claim:

1. In the formation of coatings from aqueous zein dispersions in which an alkali and a sulfonated vegetable oil are used as dispersing agents: the improvement which comprises incorporating in the dispersion lead acetate in order to increase the water resistance of the coating and reduce the time required for bringing the coating to a water-resistant state.

2. In the formation of coatings from aqueous zein dispersions in which an alkali and a sulfonated vegetable oil are used as dispersing agents: the improvement which comprises incorporating in the dispersion a substance to increase the water resistance of the coating and reduce the curing time thereof, of the group of substances consisting of the acetates and formates of alumi-

num, barium, calcium, magnesium, tin, zinc, copper and lead.

3. In the formation of coatings from aqueous zein dispersions in which an alkali and a sulfonated vegetable oil are used as dispersing agents: the improvement which comprises incorporating in the dispersion a soluble salt of a weak acid to increase the water resistance of the coating and reduce the time required for bringing the coating to a water-resistant state.

4. A coating composition which comprises: zein dispersed in water by an alkali and sulfonated taloil, said dispersion containing also lead acetate to enable a coating produced from said composition to develop a high degree of water resistance in a short period of time.

5. A coating composition which comprises zein dispersed in water by an alkali and a sulfonated vegetable oil, said dispersion containing also, to increase the water resistance of the coating formed from such composition and reduce the curing time thereof, a substance selected from the group of substances consisting of the acetates and formates of aluminum, barium, calcium, magnesium, tin, zinc, copper and lead.

6. A coating composition which comprises zein dispersed in water by an alkali and a sulfonated vegetable oil, said dispersion containing also, to increase the water resistance of the coating formed from such composition and reduce the curing time thereof, a soluble salt of a weak acid.

ALBERT L. JAMES.